

## UNITED STATES PATENT OFFICE

2,176,100

## FLUORESCENT MATERIAL AND A FLUORESCENT ELEMENT INCORPORATING THE SAME

Carl Pfanstiehl, Highland Park, Ill., assignor to Pfanstiehl Chemical Company, a corporation of Illinois

No Drawing. Application November 23, 1938, Serial No. 242,107

10 Claims. (Cl. 250—81)

This invention relates to an improved fluorescent material and a fluorescent element incorporating the same.

One of the most widely used fluorescent materials for incorporation with gaseous illuminating elements such as neon or argon, combined with mercury vapor is zinc ortho-silicate.

In my copending application Serial No. 190,880, filed February 16, 1938, is described a method for preparing zinc ortho-silicate in such manner as to improve its fluorescent properties by producing individual unground crystals of the order of one micron in cross section.

The present invention is preferably carried out in combination with the improvements therein set forth, the color of the fluorescent illumination being markedly changed by the production of fine particles of that type.

In preparing the objects of the present invention, a base comprising roughly  $1\frac{1}{2}$  molecules of zinc ortho-silicate to 1 molecule of beryllium silicate is employed.

With this is incorporated a minor percentage of an activator, such as a manganese compound, preferably manganese dioxide, and in many cases, particularly those where a white light is desired, a further minor percentage of a rare earth metal. A preferred base may be prepared by incorporating the following ingredients:

|                                 | Parts by weight |
|---------------------------------|-----------------|
| ZnO                             | 50.685          |
| BeO                             | 9.750           |
| H <sub>2</sub> SiO <sub>3</sub> | 39.565          |

This base contains approximately 3.4 molecules of zinc ortho-silicate (Zn<sub>2</sub>SiO<sub>4</sub>) to 2.2 molecules of beryllium ortho-silicate (Be<sub>2</sub>SiO<sub>4</sub>).

The ingredients are thoroughly and carefully mixed in a ball mill as described in my application Serial No. 190,880. The materials are used in the form of fine powders and mixed with a liquid such as methanol to form a paste. They are then milled in a hard porcelain ball mill with relatively light pebbles, preferably of  $\frac{1}{2}$ " to  $\frac{3}{4}$ " size, with the mill running rather slowly, so that no considerable shock will be given to the particles. The material may be milled for 20 to 22 hours. The mixture is then dried and carefully brushed through a 200 mesh screen and is then packed into a crucible for heat treating. This packing should be such as not to pack the material too tightly, or else hard sintered particles will result. The powder is then heat treated as described in my copending application Serial 190,880, in such manner that there is no sintering or

fusing of the particles, but interaction does occur. The character of material so formed should crumble readily between the fingers and require no grinding. The mixture of zinc silicate and beryllium silicate will not stand as high temperatures as zinc silicate alone and preferably the temperature should not exceed 2150° F.

To this base an activator is added. In each case, of course, the activator is added before the powder is formed and whenever it is here stated that an activator or other material is added to the base, it should be understood that it is added before formation, unless otherwise specifically stated.

When manganese is used as the activator, it is preferably employed in fairly large portions compared to the amount of manganese normally incorporated for this purpose. The addition of 0.1% of manganese gives a whitish light, but a far from brilliant one. Preferably upwards of 0.4% is employed. The use of 0.4% to 0.5% of manganese gives a whitish fluorescent illumination. The use of 4% of manganese dioxide produces an orange color and the use of 6% produces a rosy pink.

When manganese is incorporated, it is preferred to use a lower temperature, the heat treatment preferably not going over 2100° F. The degree of fluorescence increases as the manganese increases, but the color becomes more reddish. However, if higher temperatures are employed, the fluorescence becomes less and the powders produce a pink color even at the lower manganese contents.

In this connection, it should be pointed out that the colors here described do not relate to the powders themselves, but the illumination they produce under short wave radiation.

Very much improved results are obtainable by the addition of a pair of activators instead of the sole use of manganese. For this purpose any of the rare earth metals is preferred. For example, the addition to the zinc-beryllium silicate base of 0.7% of manganese dioxide and 0.4% of samarium oxide (Sm<sub>2</sub>O<sub>3</sub>) produces a very brilliant and quite white light. Very white and brilliant illumination was produced by adding to the beryllium-zinc silicate base, 1% of manganese dioxide and 0.4% to 0.5% of either samarium or neodymium oxide (Nd<sub>2</sub>O<sub>3</sub>). The use of 0.7% of manganese dioxide with 0.4% of the samarium or neodymium oxides is slightly whiter than the previous example, but it is not quite so brilliant. The use of 0.6% of samarium oxide with 0.7% of manganese dioxide is not quite so white or

bright. Less amounts than 0.4% of the rare earth metal generally give less favorable results when compared to the 0.4% to 0.5% range.

Other rare earths may be substituted for the examples given. For example, an extremely bright white light, only slightly deficient in red is produced by the use of 0.7% manganese dioxide and 0.5% lanthanum oxide in combination with the zinc beryllium base.

- 10 Many of the powders here described have a considerably greater illumination efficiency than tungsten lights. For example, the lanthanum-manganese compound described incorporating 0.7% manganese dioxide and 0.5% lanthanum oxide, used in a glass tube with half the glass covered by the powder, produces on a light meter, approximately ten times the light per unit current compared to the base tungsten lights available on the market.
- 15 20 The powder produced in accordance with this process is in the form of small unbroken crystals about 95% of which are less than two microns in size. About 50% of the crystals are from one-quarter to one micron in size.
- 25 This application is a continuation in part of my copending application Serial Number 202,804 filed April 18, 1938.

The foregoing detailed description has been given for clearness of understanding only, and no unnecessary limitations should be understood therefrom, but the appended claims should be construed as broadly as permissible in view of the prior art.

I claim:

- 30 35 1. A fluorescent powder consisting essentially of unground crystals of a size of the order of one micron in diameter of zinc beryllium silicate, the crystals containing a minor proportion of an activator.

2. A fluorescent powder comprising zinc beryllium silicate in the form of unground crystals substantially all less than two microns in size and a pair of activators, one of the activators being a rare earth metal.

3. A fluorescent element comprising unfused unground minute particles substantially all less than two microns in size of zinc beryllium silicate containing a small proportion of manganese.

4. A fluorescent material comprising zinc beryllium silicate in the form of unground crystals substantially all less than two microns in size containing approximately 0.4% to 1.0% manganese oxide and approximately 0.4% to 0.5% of a rare earth metal.

5. A material as set forth in claim 4 in which the rare earth metal is samarium.

6. A material as set forth in claim 4 in which the rare earth metal is lanthanum.

7. A material as set forth in claim 4 in which the rare earth metal is neodymium.

8. A fluorescent material comprising in the form of unground crystals substantially all less than two microns in size zinc beryllium silicate containing approximately 0.7% to 1.0% manganese oxide and approximately 0.4% to 0.5% of a rare earth metal.

9. A fluorescent material comprising minute crystals of zinc beryllium silicate containing approximately 0.4% to 1% of manganese oxide and approximately 0.4 to 0.5 of samarium.

10. A fluorescent material comprising minute crystals of zinc beryllium silicate containing approximately 0.4% to 1% of manganese oxide and approximately 0.4% to 0.5% of neodymium.

CARL PFANSTIEHL.

CERTIFICATE OF CORRECTION.

Patent No. 2,176,100.

October 17, 1939.

CARL PFANSTIEHL.

It is hereby certified that error appears in the printed specification of the above numbered patent requiring correction as follows: Page 1, second column, line 16, for the word "portions" read proportions; page 2, second column, line 24, claim 8, strike out "zinc beryllium silicate" and insert the same after "comprising", line 22, same claim; line 31, claim 9, for "0.4 to 0.5" read 0.4% to 0.5%; and that the said Letters Patent should be read with this correction therein that the same may conform to the record of the case, in the Patent Office.

Signed and sealed this 19th day of December, A. D. 1939.

(Seal)

Henry Van Arsdale,  
Acting Commissioner of Patents.

bright. Less amounts than 0.4% of the rare earth metal generally give less favorable results when compared to the 0.4% to 0.5% range.

Other rare earths may be substituted for the examples given. For example, an extremely bright white light, only slightly deficient in red is produced by the use of 0.7% manganese dioxide and 0.5% lanthanum oxide in combination with the zinc beryllium base.

- 10 Many of the powders here described have a considerably greater illumination efficiency than tungsten lights. For example, the lanthanum-manganese compound described incorporating 0.7% manganese dioxide and 0.5% lanthanum oxide, used in a glass tube with half the glass covered by the powder, produces on a light meter, approximately ten times the light per unit current compared to the base tungsten lights available on the market.
- 15 20 The powder produced in accordance with this process is in the form of small unbroken crystals about 95% of which are less than two microns in size. About 50% of the crystals are from one-quarter to one micron in size.
- 25 This application is a continuation in part of my copending application Serial Number 202,804 filed April 18, 1938.

The foregoing detailed description has been given for clearness of understanding only, and no unnecessary limitations should be understood therefrom, but the appended claims should be construed as broadly as permissible in view of the prior art.

I claim:

- 30 35 1. A fluorescent powder consisting essentially of unground crystals of a size of the order of one micron in diameter of zinc beryllium silicate, the crystals containing a minor proportion of an activator.

2. A fluorescent powder comprising zinc beryllium silicate in the form of unground crystals substantially all less than two microns in size and a pair of activators, one of the activators being a rare earth metal.

3. A fluorescent element comprising unfused unground minute particles substantially all less than two microns in size of zinc beryllium silicate containing a small proportion of manganese.

4. A fluorescent material comprising zinc beryllium silicate in the form of unground crystals substantially all less than two microns in size containing approximately 0.4% to 1.0% manganese oxide and approximately 0.4% to 0.5% of a rare earth metal.

5. A material as set forth in claim 4 in which the rare earth metal is samarium.

6. A material as set forth in claim 4 in which the rare earth metal is lanthanum.

7. A material as set forth in claim 4 in which the rare earth metal is neodymium.

8. A fluorescent material comprising in the form of unground crystals substantially all less than two microns in size zinc beryllium silicate containing approximately 0.7% to 1.0% manganese oxide and approximately 0.4% to 0.5% of a rare earth metal.

9. A fluorescent material comprising minute crystals of zinc beryllium silicate containing approximately 0.4% to 1% of manganese oxide and approximately 0.4 to 0.5 of samarium.

10. A fluorescent material comprising minute crystals of zinc beryllium silicate containing approximately 0.4% to 1% of manganese oxide and approximately 0.4% to 0.5% of neodymium.

CARL PFANSTIEHL.

CERTIFICATE OF CORRECTION.

Patent No. 2,176,100.

October 17, 1939.

CARL PFANSTIEHL.

It is hereby certified that error appears in the printed specification of the above numbered patent requiring correction as follows: Page 1, second column, line 16, for the word "portions" read proportions; page 2, second column, line 24, claim 8, strike out "zinc beryllium silicate" and insert the same after "comprising", line 22, same claim; line 31, claim 9, for "0.4 to 0.5" read 0.4% to 0.5%; and that the said Letters Patent should be read with this correction therein that the same may conform to the record of the case, in the Patent Office.

Signed and sealed this 19th day of December, A. D. 1939.

(Seal)

Henry Van Arsdale,  
Acting Commissioner of Patents.